

Oct. 13, 1959

L. PERAS

2,908,569

PROCESS OF PRODUCING SINTERED TUNGSTEN ELECTRODES

Filed Jan. 31, 1955

FIG. 1



FIG. 2



FIG. 3



FIG. 4



FIG. 6



FIG. 5



2,908,569

PROCESS OF PRODUCING SINTERED  
TUNGSTEN ELECTRODES

Lucien Peras, Billancourt, France, assignor to Regie Nationale des Usines Renault, Billancourt, France

Application January 31, 1955, Serial No. 485,180

Claims priority, application France February 5, 1954

1 Claim. (Cl. 75—207)

This invention relates to improvements in spark plugs, more particularly to spark plugs for internal combustion engines.

The invention relates to a new constructional form of spark plugs which are very suitable for ignition by capacity discharge and whose working life is much greater than that of spark plugs which have been constructed heretofore, and of the same order as the life of the currently used high voltage spark plugs.

The spark plugs according to the present invention are constituted by co-axial circular electrodes machined from special alloys, the dimension of the electrodes being much greater than that of the region subjected to the sparks. The metals from which the electrodes are machined are alloys rich in tungsten obtained by impregnation of calcined tungsten bodies of carefully adjusted porosity by another metal or alloy having particular properties which is brought to a molten condition for the impregnation process. The tungsten content of the alloys which are suitable is comprised between 65% and 95%. According to the invention, the complementary metal added by impregnation in the molten condition can be:

pure silver,  
pure palladium,  
palladium-silver alloys in any proportions.

A moderate melting temperature of less than 1,400 degrees centigrade permitting of the easy impregnation of the tungsten body is reconciled with good properties of resistance to the spark by using alloys containing 70% palladium and 30% silver, or else 50% palladium and 50% silver.

For example, in tests carried out on a vehicle having a gasoline engine of current construction, wherein the ignition of the four 748 cm.<sup>3</sup> cylinder engine is effected by low voltage (800 to 1,000 volts approx.). The life-distance of the spark plugs as hitherto used was scarcely more than 5,000 kilometres.

With a spark element wherein the electrodes, spaced from one another by 0.12 mm. by mica whose mechanical action is reinforced by an insulating cement, are formed of an alloy consisting of 85% tungsten and 15% silver, it was possible to travel 18,000 kilometres with the same vehicle under the same running conditions as those in the preceding test before it was necessary to change the spark plugs. The distance travelled could have been increased to 25,000 kilometres with another set of spark plugs wherein the electrodes consisted of an alloy of 80% tungsten, 9.8% palladium and 4.2% silver. In both cases the spark element was held in a mounting which enabled ordinary high voltage spark plugs to be fitted at the appropriate place and time, the peripheral electrode being connected to the frame by its entire outer surface and the central electrode being held at its center by a spindle which is in turn connected to the other pole of the current source.

With a view to reducing costs, it is possible to reduce the height of the spark element to, for example, 3 mm.

and to braze each of the electrodes end-on to a conducting member of, for example, steel.

Several constructional forms of spark plugs particularly suitable for electrodes according to the invention are shown in partial axial section in the accompanying drawings purely by way of example.

Figs. 1 through 5 are fragmentary sectional views of spark plugs according to the invention,

Fig. 6 is an elevation view of a spark plug element partly in section.

Figs. 1 and 5 show a spark plug comprising electrodes 1, 2 with insulating material 3 which is for example cement vitrified into position or cement, consisting of a refractory mineral charge agglomerated by a heat-hardened organic substance, and a mica ring 4 arranged at the height of the region where the sparks are produced. The mica ring protects the insulating material and supports the fire of the spark.

In other constructional forms (see Figs. 2, 3 and 4), 20 a circular swelling or curvature 5 can be formed at the top of one of the cylindrical electrodes in such manner that the shortest distance between electrodes is outside the insulating material and that the spark, jumping beyond the said insulating material, does not damage it.

25 In another possible constructional form based on prolonged tests, electrodes of pure tungsten were employed provided that the volume of pure tungsten was substantially greater than that which is subjected to the spark.

For example, it would not be advantageous to cause 30 the spark to jump between two tungsten toruses each constituted by a wire placed in the form of a circle and secured by brazing to a cylindrical steel part. The electrodes formed in this known manner can provide, for example in motor cars, only a quite inadequate service life, 35 even if the diameter of the tungsten wire is at the upper limit of approx. 0.25 mm. permissible for winding and brazing to a steel ring whose thickness is of the order of 0.6 mm.

In order to define precisely the features of the invention, reference will now be made to the example of a 40 spark plug element (Fig. 6) for a gasoline engine. The electrodes 1 and 2 are connected respectively to the electric generator (not shown) by the crown 6 and the cylindrical stem 7. The two electrodes are insulated from 45 one another and held in position by the cement 3. The spark controlled by the distributor jumps at any point in the inter-electrode space between two points such as A and B situated on the same diameter.

Whereas the small toroidal surfaces which have to be 50 subjected to the spark, taken in section at A and B through the plane of the drawing, have a width not exceeding 0.1 mm., the tungsten electrodes used by way of example and in accordance with the invention have a thickness of 1 mm. and a height of 5 mm. According 55 to the invention, no material discontinuity of the brazed connection, for example, must exist within each of the electrodes at less than 2 mm. from the line of sparking.

In order that the service life of the electrodes should 60 fulfill the requirements of, for example, automotive use, the tungsten must not be porous and its compactness should be such that its specific weight should be greater than 17.5 g./cm.<sup>3</sup> and preferably greater than 18 g./cm.<sup>3</sup>. This condition is difficult to fulfill since the only tungsten products commercially obtainable which exhibit no 65 porosity are those wires whose manufacture has included the preparation of a rod by calcining, then a hammering and a series of wire-drawings, which are mechanical treatments to which spark plug electrodes cannot be subjected during manufacture in view of their form and their size.

The invention also relates to a method of preparing 70 pure tungsten electrodes for spark plugs operating with

capacity discharge, having the compactness necessary for good operation in practice. It comprises the following conditions taken necessarily in combination:

Use of a pure tungsten powder of sufficient fineness for the specific weight of the rammed powder to be less than 3 g./cm.<sup>3</sup>.

Shaping by moulding under pressure, preferably by double compression in a floating matrix, the moulding pressure being greater than 7 kg./mm.<sup>2</sup> although low enough to prevent the appearance of cracks in the moulded article. A suitable pressure is one between 7 and 10 kg./mm.<sup>2</sup>.

Calcining at a temperature of between 1,800 and 2,100° C. by heating in a graphite resistance furnace in an atmosphere consisting of a mixture of argon and hydrogen, the hydrogen content being less than 10%. In another embodiment it is possible to place the compressed article to be sintered in a cold furnace, heat to 1,100° in an atmosphere of pure hydrogen, stop the current of hydrogen at this instant and substitute therefor a current of pure argon. It is sufficient to maintain this temperature for 15 to 30 minutes.

Sintering can be carried out by heating the powder electrode in an atmosphere of pure hydrogen up to a temperature between 1,000° centigrade and 1,300° centigrade and then in an atmosphere of argon up to a maximum temperature of 2,100° centigrade.

The hydrogen is necessary for ensuring good connection between the grains of tungsten, probably because it effects the reduction of oxide traces which may cover the metallic grains. It has been found, moreover, that the use of hydrogen at too high a temperature and in too

strong a content has the result of carburizing the tungsten (probably through the intermediary of gaseous hydrocarbons formed by the action of the hydrogen on the graphite of the furnace) and of making it fragile, unmachinable and of low resistance to sparking.

The electrodes are then machined to their final size.

I claim:

The process of making low voltage discharge device electrodes, which comprises, providing pure tungsten powder having a specific weight less than three grams per cubic centimeter, molding the powder into electrodes in a matrix under pressure between the limits of seven kilograms per square centimeter and ten kilograms per square centimeter, heating the electrodes in the presence of pure hydrogen to a temperature between 1000° centigrade and 1300° centigrade and then heating them to approximately 2100° centigrade in the presence of argon thereby to form non-porous electrodes.

References Cited in the file of this patent

UNITED STATES PATENTS

|           |                |                |
|-----------|----------------|----------------|
| 2,008,617 | Lampitt        | July 16, 1935  |
| 2,069,951 | Hastings       | Feb. 9, 1937   |
| 2,253,533 | Ruben          | Aug. 26, 1941  |
| 2,311,647 | Doran          | Feb. 23, 1943  |
| 2,491,866 | Kurtz          | Dec. 20, 1949  |
| 2,578,754 | Smits          | Dec. 18, 1951  |
| 2,625,922 | Smits          | Jan. 20, 1953  |
| 2,675,310 | Hall           | Apr. 13, 1954  |
| 2,689,556 | Smits          | Sept. 21, 1954 |
| 2,712,685 | Johnson et al. | July 12, 1955  |
| 2,791,022 | Stuermer       | May 7, 1957    |